

Feb. 25, 1969

LARS-GUNNAR BERGH

3,429,055

METHOD FOR HEAT TREATMENT

Filed Feb. 12, 1968

Sheet 1 of 2

FIG. 1.



FIG. 2.



INVENTOR:  
LARS GUNNAR BERGH  
BY *Howard & Howard*  
ATTYS.

Feb. 25, 1969

LARS-GUNNAR BERGH

3,429,055

METHOD FOR HEAT TREATMENT

Filed Feb. 12, 1968

Sheet 2 of 2

FIG.3.



FIG.4.



INVENTOR  
LARS GUNNAR BERGH

*Houston & Houston*

ATTYS.

**1**

3,429,055

**METHOD FOR HEAT TREATMENT**

Lars-Gunnar Bergh, Bankeryd, Sweden, assignor to Aktiebolaget Svenska Flaktfabriken, Stockholm, Sweden  
Continuation-in-part of application Ser. No. 606,458, 5  
Dec. 30, 1966. This application Feb. 12, 1968, Ser.  
No. 709,856

Claims priority, application Sweden, Sept. 16, 1963,  
10,102/63

U.S. Cl. 34—13.8 2 Claims  
Int. Cl. F26b 3/04; B29j 5/00

**ABSTRACT OF THE DISCLOSURE**

A method for heat treatment of dry fibre boards in which the heating medium is blown perpendicularly against the boards and is maintained between 160° C. and 235° C. to heat the boards and at the same time prevent local overheating in random areas due to exothermic reactions occurring within the boards.

The present application is a continuation-in-part of my application No. 606,458 filed Dec. 30, 1966 as a continuation of my earlier application S.N. 360,302 filed 25 Apr. 16, 1964, both now abandoned.

The present invention relates to a method for the heat treatment of dry wood fibre boards or similar material and more particularly the treatment by hot air at temperatures exceeding 160° C.

An important object of the invention is to prevent a harmful overheating of the dry wood fibre boards or similar material during the heat treatment.

Other objects and a more detailed understanding of the invention may be had by referring to the following description and claims, in conjunction with the accompanying drawings in which:

FIG. 1 is graphical representation showing the relationship between the swelling and the heating time at various temperatures of typical wood fibre boards;

FIG. 2 is a graphical representation showing the relationship between the moisture absorption and the heating time at various temperatures of typical wood fibre boards;

FIG. 3 is a vertical section through a heat treatment apparatus constructed in accordance with the present invention; and

FIG. 4 is a longitudinal section taken along the line 4—4 in FIG. 3.

Compressed wood fibre boards, for example hardboards, are heat-treated or hardened in their dry state in order to impart to them certain properties of strength, water absorption, swelling, etc. This heat treatment is usually carried out with the aid of hot air, which is maintained in circulation around the boards. If the heat treatment is to produce the desired effect, it must be carried out at a high temperature above 160° C. At a temperature of approximately 140° C. an exothermic reaction occurs in dry wood fibre board which gradually increases the temperature of the board above that of the ambient air. To prevent the temperature of the board from rising high enough to cause charring and ignition which occurs at approximately 235° C., I have found that the circulating air must have a certain cooling effect. In conventional heat-treating equipment (both of the continuous and chamber types) a parallel flow of air at a temperature of 160 to 165° C. is used. Investigations have proved that a certain relationship exists between the effects of treatment temperature and time. The diagrams in FIGS. 1 and 2 show the relationship between time, temperature and increase in thickness due to swelling and water ab-

sorption, and that for a constant time, both swelling and absorption will decrease with increasing temperature.

The present invention is based on the discovery that the present high demands for quality properties in the above stated respects cannot be met by a conventional treatment in known apparatus, operating with parallel flow of treatment medium along the surface of the boards, since the high temperatures necessary to fulfill the said requirements could not be used in this apparatus without the risk of ignition and fire. The risk of ignition and fire is too great, because a completely uniform air distribution is never obtained in said known apparatus, and, within reasonable pressure limits, only a relatively low heat transmission coefficient between air and boards is attained. The heat transmission coefficient is of decisive importance after the exothermic reaction has set in and, for control of the temperature gradient in the board, it is necessary to maintain as low a temperature difference as possible between board and air. The quantity of heat to be supplied for heating the board to the required temperature and the quantity of heat which then must be removed after the board has been brought to the treatment temperature is dependent on the product of the heat transmission coefficient and the temperature difference between board and air. A high heat transmission coefficient permits a short heating-up time and a small temperature difference when the board has reached the treatment temperature.

In the method of the present invention, a high heat transmission coefficient is obtained while a harmful increase in the exothermic reaction occurring in the boards is prevented, by supplying hot air of regulated temperature in the form of uniformly spaced jets at a high velocity and substantially at right angles against both sides of the boards. In this manner, with the same pressure loss (10–40 mm. Hg) the heat transmission coefficient value is approximately five times that obtained by supplying the air in the form of parallel streams. My invention is accompanied by other advantages. It provides a very uniform air distribution across the board, both in the lengthwise and crosswise directions. This is even more pronounced, if the board is kept in motion at right angles in relation to the discharged direction of the air jets during the treatment process; the movement can be continuous, progressive or oscillating. In this manner, local excessive temperature in the board is avoided. The risk of the occurrence of partial excessive temperature is especially great at the so-called flash or burr, i.e., the uneven edge portions arising outside the pressing plate during the pressing. With a treatment according to the invention, it is therefore advisable that this flash is removed before heat treatment. With right-angle blowing, boards have been treated at a temperature of 215° C. for a period of six hours without ignition taking place. In the areas where the exothermic reaction occurs, the temperature of the board is then only about 5° above that of the air. A completely satisfactory result was obtained after a treatment time of only 30 minutes, which means that there is an adequate margin of safety as regards ignition. The treatment time can be varied within wide limits depending on the properties it is desired to impart to the treated board.

This invention is applicable to dry boards, i.e., boards in which there is no free moisture and in which the hygroscopic moisture is at a minimum. The drawing illustrates an apparatus for carrying the method into practice. The apparatus consists of a treatment channel provided with elements for the transport of the boards and equipped with elements for heating and circulation of the treatment medium. Characteristic of the apparatus is that air distribution boxes are arranged on both sides of each transport plane and the walls of these boxes facing the

transport plane are provided with a large number of evenly-spaced discharged openings for blowing-on treatment medium in the form of jets substantially directed at right angles to the dry boards.

In the apparatus shown in FIG. 3, an outer housing 1 of the apparatus has inspection panels or doors 2. Blower boxes 3 and 4 are mounted in the housing from which air is blown through slots or perforated plates at right angles, or possibly slightly inclined, against the material 11. The material is supported on rollers 5 mounted in bearings 6 and driven by means of sprockets 7 and chains (not shown). Circulation of air in the apparatus is produced by a fan 8 driven by a motor 9. When the air strikes the material, it is deflected sideways and is returned through the ducts 17 and 18 to the circulating fan 8. The quantity of heat necessary for the heating-up period is supplied by heaters 10. These could suitably (with regard to the relatively high air temperature being used) be supplied with hot oil from a source of heat (not shown). Circulating air can also be heated by means of air from an oil-fired heat exchanger; possibly it is conceivable that flue gases could be used directly. During heat treatment, gases are generated, some of which are poisonous (CO) and the housing must therefore be ventilated. This takes place through a flue 12 fitted with a controllable damper 13. The location of the fan shown in FIG. 3 provides the advantage that the static pressure on the housing of the apparatus is low. It can even be negative in relation to the static pressure outside the housing of the apparatus. This makes the risk of external leakage very small. The apparatus is supported by a stand 14. FIG. 4 shows that the upper blower box, which is located nearest to the material, is fitted with normal perforations 15, and the lower box, which must be located further away from the track due to the rollers 5, is fitted

10  
15  
20  
25

with nozzles 16. The apparatus may also be fitted with double rollers, if desired, in which case both of the blower boxes 3 and 4 are fitted with nozzles.

I claim:

1. A method of heat-treating dry hardboards of wood fibre and the like which are subject to localized overheating in random areas due to exothermic reactions occurring within the boards at temperatures above 140° C., and are subject to charring at temperatures above 235° comprising the steps of:

supplying air at a temperature exceeding 160° C. and below 235° C. where charring starts, and directing said supplied air in the form of uniformly-spaced jets at high velocity substantially at right angles against both sides of the boards, said air serving to heat the boards up to a temperature approximating the temperature of the air and serving to cool said random areas of localized overheating wherein the board temperature has started to rise above said air temperature.

2. A method according to claim 1 wherein said dry hardboards have an absence of free moisture and in which the hygroscopic moisture is at a minimum.

#### References Cited

#### UNITED STATES PATENTS

|           |         |                 |       |            |
|-----------|---------|-----------------|-------|------------|
| 835,843   | 11/1906 | Baetz           | ----- | 34—13.8 XR |
| 2,591,621 | 4/1952  | Shegda          | ----- | 34—160 XR  |
| 3,099,541 | 7/1963  | Hildebrand      | ----- | 34—23 XR   |
| 3,199,213 | 8/1965  | Milligan et al. | ----- | 34—13.8    |

KENNETH W. SPRAGUE, Primary Examiner.

U.S. Cl. X.R.

35 34—23